

# United States Patent Office

2,984,552

Patented May 16, 1961

1

2,984,552

LEADED GASOLINE CONTAINING PHOSPHORUS  
Everett N. Case, Homewood, Ill., assignor to Sinclair  
Refining Company, New York, N.Y., a corporation of  
Maine

No Drawing. Filed Nov. 19, 1957, Ser. No. 697,318  
2 Claims. (Cl. 44—69)

My invention relates to improved gasoline which is of high octane number and which contains tetraethyl lead as an anti-knocking agent.

By and large, modern gasolines for use in spark-ignited internal combustion engines have an octane number of at least 85 RON, that is, as determined by the Research Method, and they contain tetraethyl lead, generally within the range from 0.5 to 3.0 cc. per gallon, or even as much as approximately 4.5 cc. per gallon, as a knock-suppressing agent. Tetraethyl lead is the most widely used anti-knock agent, and is very effective for this purpose, but it suffers from the defect that it causes lead-containing deposits in the cylinders. These deposits have a tendency to cause preignition; that is, the deposits are hot and cause the mixture in the cylinder to burn before combustion is initiated at the proper time by the spark plug. Preignition can be controlled, as the art is aware, by the addition of phosphorus additives to leaded gasoline. However, the phosphorus additive must be properly chosen or otherwise when the engine is put into service and operated, the octane requirement increase encountered as the engine cylinders build up deposits will be greater than that which takes place when no phosphorus additive is used.

In accordance with my invention, yellow phosphorus (sometimes known as white phosphorus or alpha-white phosphorus) is incorporated into leaded gasoline with the result that preignition is suppressed and the octane requirement increase as the engine is used is less than that encountered with the base fuel, that is, the gasoline not containing any phosphorus additive. The yellow phosphorus is incorporated into the gasoline generally in the amount of from 0.1 to 2 theory, and preferably in the amount of from 0.2 to 0.6 theory, 1.0 theory meaning that for each three gram atoms of lead present in the tetraethyl lead there are present two gram atoms of yellow phosphorus. One theory is based upon the premise that the phosphorus and the lead in the tetraethyl lead react in the combustion zone to form lead orthophosphate,  $Pb_3(PO_4)_2$ . Stated somewhat differently, for each three gram moles of tetraethyl lead present in the gasoline, there is also generally present from 0.2 to 4 gram atoms of yellow phosphorus and preferably from 0.4 to 1.2 gram atoms of yellow phosphorus.

### Example

As a specific illustration of the practice of my invention, there was first obtained a sample of base gasoline which was composed of a major amount of heavy reformate from straight run naphtha and a minor amount of light fluid cracked gasoline. The base gasoline contained 3 cc. per gallon of tetraethyl lead together with the usual scavengers and had an API gravity of 39.2. The base gasoline, when containing the tetraethyl lead, had an octane number of 103.1 by the Research Method and an octane number of 91.1 by the Motor Method. The ASTM distillation of the gasoline was as follows:

|                       | ° F. |
|-----------------------|------|
| Initial boiling point | 115  |
| 10 percent            | 210  |
| 50 percent            | 324  |
| 90 percent            | 357  |
| End point             | 421  |

2

Into a portion of the base gasoline there was dissolved 0.3 theory of yellow phosphorus, this amount being 0.0936 gram of yellow phosphorus per gallon of base gasoline. When the base gasoline and the base gasoline containing the yellow phosphorus were subjected to comparative tests in a spark-ignited single cylinder combustion engine, it was found that the gasoline containing the yellow phosphorus showed a ping count per hour of 157 and that the base gasoline showed a ping count per hour of 333.

A second sample of base fuel was obtained, this particular sample being composed of a mixture of alkylate, heavy reformate from straight run naphtha, light fluid cracked gasoline and butane. This particular gasoline contained 3 cc. per gallon of tetraethyl lead together with the usual scavengers, had an API gravity of 53.6, an octane number by the Research Method of 101.4 and an octane number by the Motor Method of 91.4. The ASTM boiling range of the second base gasoline was as follows:

|                       | ° F. |
|-----------------------|------|
| Initial boiling point | 90   |
| 5 percent             | 118  |
| 50 percent            | 264  |
| 90 percent            | 319  |
| End point             | 381  |

Into a portion of the second base gasoline there was dissolved yellow phosphorus in the amount of 0.3 theory. The second base gasoline and a portion thereof containing the yellow phosphorus were then tested in a 1957 model automobile engine for octane requirement increase, with the results shown in the table below:

### Engine octane requirement

| Hours                       | Base            |                 | Base+0.3 Theory P |                 |
|-----------------------------|-----------------|-----------------|-------------------|-----------------|
|                             | 1,500<br>r.p.m. | 2,500<br>r.p.m. | 1,500<br>r.p.m.   | 2,500<br>r.p.m. |
| 40                          |                 |                 |                   |                 |
| Start (clean)               | 94              | 93              | 93                | 93              |
| 42                          | 98              | 97              | 99                | 97              |
| 84                          | 100             | 100             | 100               | 98              |
| 126                         | 102             | 102             | 100               | 99              |
| 168                         | 103             | 103             | 101               | 99              |
| 210                         | 103             | 103             | 101               | 99              |
| Octane Requirement Increase | 9               | 10              | 8                 | 6               |

### I claim:

1. Gasoline containing from 0.5 to 4.5 cc. per gallon of tetraethyl lead and also containing yellow phosphorus in the amount of from 0.1 to 2 theory.
2. Gasoline containing from 0.5 to 4.5 cc. per gallon of tetraethyl lead and also containing yellow phosphorus in the amount of 0.2 to 0.6 theory.

### References Cited in the file of this patent

#### UNITED STATES PATENTS

|           |                |               |
|-----------|----------------|---------------|
| 1,913,970 | Albers         | June 13, 1933 |
| 2,405,560 | Campbell       | Aug. 13, 1946 |
| 2,563,101 | Colwell et al. | Aug. 7, 1951  |
| 2,794,717 | Gilbert        | June 4, 1957  |
| 2,797,153 | Bereslavsky    | June 25, 1957 |

#### FOREIGN PATENTS

|           |               |                |
|-----------|---------------|----------------|
| 709,653   | Great Britain | June 2, 1954   |
| 1,094,828 | France        | May 24, 1955   |
| 1,123,123 | France        | Sept. 18, 1956 |

#### OTHER REFERENCES

- 70 "Petroleum Refining With Chemicals," by Kalichevsky et al., Elsevier Publishing Co., 1956, p. 491.